

Aug. 1, 1972

S. W. K. SHAW ET AL

3,681,059

NICKEL-CHROMIUM ALLOY FOR REFORMER TUBES

Filed Dec. 12, 1969

5 Sheets-Sheet 1



INVENTORS  
STUART WALTER KEE SHAW  
BY PETER JOHN PENRICE

M. D. Purcell

ATTORNEY

Aug. 1, 1972

S. W. K. SHAW ET AL

3,681,059

NICKEL-CHROMIUM ALLOY FOR REFORMER TUBES

Filed Dec. 12, 1969

5 Sheets-Sheet 2



INVENTORS  
Stuart Walter Ker Shaw  
Peter John Fenrice  
BY

M. L. Pineel  
ATTORNEY

Aug. 1, 1972

S. W. K. SHAW ET AL

3,681,059

NICKEL-CHROMIUM ALLOY FOR REFORMER TUBES

Filed Dec. 12, 1969

5 Sheets-Sheet 3

25% Cr, 2% Nb



Ti □. H.

25% Cr, 3% Nb



Ti □. 4.

INVENTORS  
STUART WALTER KER SHAW  
BY PETER JOHN PENRICE

M. L. / J. J.

10/16/72

Aug. 1, 1972

S. W. K. SHAW ET AL

3,681,059

NICKEL-CHROMIUM ALLOY FOR REFORMER TUBES

Filed Dec. 12, 1969

5 Sheets-Sheet 4

30% Cr, 2% Nb



Ti Q.S.

30% Cr, 3% Nb



Ti Q.S.

INVENTORS  
STUART WALTER KER SHAW  
PETER JOHN PENRICE

BY

M. L. Purcell  
ATTORNEY

Aug. 1, 1972

S. W. K. SHAW ET AL

3,681,059

NICKEL-CHROMIUM ALLOY FOR REFORMER TUBES

Filed Dec. 12, 1969

5 Sheets-Sheet 5



INVENTORS  
STUART WALTER KER SHAW  
PETER JOHN PEYRICE

BY

M. L. Pinel  
ATTORNEY

3,681,059

## NICKEL-CHROMIUM ALLOY FOR REFORMER TUBES

Stuart Walter Ker Shaw, Coldfield, and Peter John Penrice, Birmingham, England, assignors to The International Nickel Company, Inc.

Filed Dec. 12, 1969, Ser. No. 884,670  
Claims priority, application Great Britain, Dec. 13, 1968,

59,479/68

Int. Cl. C22c 19/00

U.S. Cl. 75—134 F

5 Claims

### ABSTRACT OF THE DISCLOSURE

Carbide-strengthened alloy containing nickel, chromium, molybdenum and/or tungsten, cobalt and niobium provides combination of high stress-rupture strength at elevated temperatures, resistance to corrosion by combustion products of hydrocarbon fuels, good weldability and good castability and is particularly satisfactory for use in production of gas plant apparatus, such as reformer tubes.

The present invention relates to nickel-chromium alloys for use at high temperatures and more particularly to carbide-strengthened nickel-chromium alloys.

Many industrial processes, for instance, the "reforming" of hydrocarbons, are now carried out at temperatures of up to 1000° C. and above require plant apparatus and articles made of alloys that will withstand stress and corrosive attack at these temperatures. Alloys for such use should have good casting properties, especially for casting in air, so that components of the plant can be economically produced by casting, and should also be weldable.

In the reforming process hydrocarbons react with steam in the presence of a catalyst to form a mixture of hydrogen and carbon monoxide and this gas mixture is widely used, under the name "synthesis gas," for the production of alcohol. It is also used as a source of hydrogen for ammonia production. The reforming reaction is carried out at high temperatures, e.g., from 800° C. to 1000° C., under elevated pressure in tubular reactors known as reformer tubes, which are heated externally by the combustion of hydrocarbon fuels.

Alloys for reformer tubes must have good resistance to creep and rupture under stress at the operating temperatures and must maintain adequate toughness when heated for prolonged periods. Reformer tube alloys must resist carburization and also corrosion by the combustion products of impure fuels, which can cause sulphidation attack on some alloys. Hitherto, reformer tubes have usually been made, by centrifugal casting, from 25% Cr-20% Ni steels (known by the Alloy Casting Institute designation "HK"), though higher nickel alloys are being considered for this use.

Although many attempts have been made to overcome the foregoing problems and others, there is still a need for alloys having an improved combination of high stress-rupture strength along with satisfactory corrosion resistance, weldability and castability for production of reformer tubes.

There has now been discovered an air-castable nickel-chromium alloy containing a specially controlled combination of carbon, carbide-forming elements and matrix elements which provides highly desirable strength, including stress-rupture strength and impact strength, along with good corrosion resistance for service in apparatus which must withstand long-time usage in corrosive environments at elevated temperatures, including gas reforming plant apparatus and other apparatus, e.g., glass-forming apparatus.

It is an object of the present invention to provide a nickel-chromium alloy having high strength and good corrosion resistance, particularly including resistance to detrimental carburization.

Another object of the invention is to provide high strength corrosion-resistant articles and structures, including castings, welded structures, reformer tubes and also spinners or spinnerettes for production of glass fibers.

Other objects and advantages will become apparent from the following description taken in conjunction with the accompanying drawing in which:

FIG. 1 is an alloy chart having total percentages of percent molybdenum plus one-half times percent tungsten along the ordinate axis and percentages of chromium along the abscissa axis and illustrating specially correlated molybdenum and/or tungsten-chromium areas

ABCDEFA

and GHIJKLMNOP.

FIG. 2 is an alloy chart having percentages of cobalt along the ordinate axis and percentages of chromium along the abscissa axis and illustrating, inter alia, specially correlated cobalt-chromium areas MUVOPQM, MNOPQM and RSOTUR.

FIGS. 3 through 8 are charts depicting stress-rupture life, in hours, in relation to alloy composition proportions, e.g., percentages of cobalt, or niobium or total percentage of percent molybdenum plus one-half the percent tungsten.

Generally speaking the present invention contemplates an alloy containing 0.4% to 1.4% carbon, 0.5% to 5% niobium, 23.5% to 33% chromium, one or both of molybdenum and tungsten in amounts so correlated with the chromium content that the sum (percent Mo)+½ (percent W) is 1% to 9% and the composition of the alloy is represented by a point within the area ABCDEFA in FIG. 1 of the accompanying drawing, cobalt in an amount from 5% to 42% so correlated with the chromium that the composition of the alloy is represented by a point within the area MUVOPQM in FIG. 2 of the accompanying drawing, up to 12% iron, up to 1% in total of titanium or aluminum or mixtures thereof, up to 1% zirconium and up to 0.1% boron. The balance of the composition, apart from impurities and incidental elements, is nickel. Alloy composition percentages referred to herein are by weight percent.

The high strength of the alloy at elevated temperatures is largely due to the presence of insoluble carbides. Carbon is therefore an essential constituent of the alloy, and for adequate stress-rupture strength at least 0.4% carbon must be present. As the carbon content is increased the stress-rupture strength at first increases but then decreases. Excessive amounts of carbon must also be avoided because as the carbon content increases the impact strength of the alloys decreases and advantageously the carbon content does not exceed 1%. The optimum carbon content depends on the manner in which the castings are made.

In industrial practice, reformer tubes are made by centrifugal casting in a metal mould preheated to 200° C. to 400° C. These casting conditions result in undirectional solidification radially inwards from the mould face, which promotes columnar crystallization, and the formation of a uniform dispersion of fine carbide particles. For castings made in this way, and also for those made by static chill-casting, the best combination of stress-rupture and impact strengths is obtained with carbon contents of 0.43% to 0.7%. In contrast to this the carbide particles in castings made in sand or other refractory moulds, where cooling takes place more slowly, are much coarser. Thus a higher carbon content is generally required to achieve a given stress-rupture life in such a casting than in a chill-cast casting and optimum properties are obtained with

from 0.6 to 0.8% carbon. However the alloys are cast, if they are to be welded under conditions of very severe restraint, the carbon content should be as low as is consistent with the strength required, and is desirably less than 0.65%.

Niobium also contributes to the stress-rupture strength as a carbide-former, and at least 0.5% and advantageously at least 1% is present for this purpose. As the niobium content increases the stress-rupture strength passes through a maximum and then begins to fall. Hence the niobium content must not exceed 5%, and more usefully it is not more than 4%. Most advantageously the niobium content is 1.5% to 3.5% to obtain high stress-rupture strength.

Tantalum may be introduced incidentally with the niobium in an amount up to one-tenth of the niobium content, but larger amounts of tantalum very adversely affect the stress-rupture life.

Chromium in the alloys confers resistance to corrosion, but to avoid the formation of an undesirable alpha-chromium phase the chromium content must not exceed 33%.

Tungsten and molybdenum contribute to the stress-rupture strength of the alloy. The combined molybdenum-tungsten content, expressed as percent  $Mo+\frac{1}{2}$  (percent W), must be at least 1%. As this content is increased at the expense of nickel in an alloy of otherwise fixed composition, the stress-rupture strength increases to a maximum and then falls. The value of percent  $Mo+\frac{1}{2}$  (percent W) at which this maximum is reached is inversely related to the chromium content, as indicated by the shape of the area ABCDEFA in FIG. 1. Advantageously, the value of percent  $Mo+\frac{1}{2}$  (percent W) is at least 2%, and is so correlated with the chromium content that the composition of the alloy corresponds to a point within the area GHJKLG.

At a given combined content of molybdenum and tungsten, the stress-rupture life also depends upon the relative proportions of molybdenum and tungsten, and beneficially the alloys contain at least 2% of tungsten.

Cobalt also contributes to the stress-rupture life, which rapidly increases to a maximum as the cobalt content increases in an alloy having the optimum combined molybdenum and tungsten content for given contents of chromium and niobium, and then decreases as the cobalt is further increased. The cobalt content at which the best properties are obtained increases with the chromium content, as indicated by the shape of the area MUVPQM in FIG. 2, and advantageously the composition of the alloys corresponds to a point in the area MNOPQM and most advantageously to a point in the area RSOTUR.

The alloys may contain small amounts of titanium or aluminum or both, up to a maximum of 1% in total. Titanium in these amounts has an advantageous effect on the tensile ductility provided the alloy is cast in such a way, e.g., centrifugally cast, that oxide inclusions are avoided, and aluminum does not impair the properties. Thus, centrifugally-cast tubes can contain up to 1% of titanium or aluminum, but statically-cast castings, which are more prone to oxide film entrapment, are preferably substantially free from these elements. In such castings any amounts of titanium and aluminum introduced from scrap or as deoxidants should be kept below 0.5%.

Small additions of zirconium also benefit the tensile ductility and stress-rupture life of the alloys, and both zirconium and boron improve the ratio of notched to plain (unnotched or smooth-bar) tensile strength. It has also surprisingly been found that additions of zirconium improve both the weldability of the alloys and the stress-rupture life of the weld metal deposited from filler material of matching composition. For these purposes the alloys can contain up to 1% zirconium and 0.1% boron, for example from 0.005% to 0.5% zirconium and 0.001% to 0.05 boron. Advantageously, the matching filler material has a higher zirconium content than the component being welded.

Of the impurities and incidental elements such as residual deoxidants commonly found in nickel-chromium alloys for use at high temperatures, silicon and manganese may be present in amounts up to 2% each, but the contents of these elements preferably do not exceed 1% each.

The alloys are advantageously deoxidized by means of an addition of magnesium, e.g., as a nickel-15% magnesium master alloy, leading typically to a residual magnesium content of 0.01% to 0.02% or 0.04%. Such residual magnesium contents improve the tensile ductility of the alloys. Nitrogen, which is introduced when the alloys are air-melted, may be present in amounts up to 0.15%.

Iron, which may be introduced incidentally as a constituent of ferro-alloys used as a source of other alloying elements, may be present in amounts up to 12%, though it generally impairs the stress-rupture life, and for the best properties the iron content should not exceed 0.5% and is preferably as low as possible. However quite satisfactory results are obtained with amounts of iron up to 5%, e.g., from 2% to 4%, which enable the alloys to be produced at desirable low costs allowing niobium, tungsten and molybdenum to be introduced as ferro-alloys.

Two advantageous alloys according to the invention contain amounts of chromium, cobalt, molybdenum and tungsten in the following combinations of ranges:

- (a) 24% to 27% chromium, 8% to 20% cobalt, and at least 5% tungsten, with percent  $Mo+\frac{1}{2}$  (percent W) from 4% to 7%; or,
- (b) 28% to 32% chromium, 20% to 30% cobalt, and at least 4% tungsten, with percent  $Mo+\frac{1}{2}$  (percent W) from 2% to 4%.

The composition of each of these alloys also advantageously corresponds to points within the areas GHJKLG and RSOTUR in FIGS. 1 and 2, respectively. They also contain 1.5% to 3.5% niobium, most advantageously 1.5% to 2.5% niobium, and 0.4% to 0.8% carbon. Within this range, the most beneficial carbon content depends on the manner of casting, as explained herein and should be lower than 0.65% if weldability under severe restraint is of importance. Beneficially the alloys also contain one or both of titanium and zirconium, e.g., 0.03% to 0.2% titanium and 0.005% to 0.3% zirconium.

An especially advantageous composition is about 25% chromium, about 12% cobalt, about 9% tungsten, about 0.5% molybdenum, about 2% niobium, either about 0.1% titanium or about 0.01% zirconium and about 3% iron. The carbon content is normally 0.5% for centrifugally cast tubes and 0.65% for said or other refractory mould castings; the balance, apart from impurities, being nickel.

Numerous tests made on alloys of different compositions have shown that in order to obtain a good combination of satisfactory properties it is important that the contents of the constituents of the alloys are correlated according to the invention.

The alloys used in the tests were prepared by air-melting with a conventional addition of 0.3% manganese, 0.3% silicon and 0.03% calcium or magnesium (added as calcium-silicide or nickel-magnesium) as deoxidants, and cast as test-pieces in investment moulds.

Results of such tests are illustrated graphically in FIGS. 3 to 8 of the accompanying drawings and are set forth in the tables.

In FIGS. 3 to 8 the stress-rupture life in hours determined under a stress of 3 ton f./in.<sup>2</sup> (2240-pound long tons per square inch) and at a temperature of 1000° C., is plotted on a logarithmic scale against the value of percent  $Mo+\frac{1}{2}$  (percent W). FIGS. 3 and 4 relate to alloys nominally containing 25% chromium and 0.75% carbon and show the effect of varying the cobalt content, at 2% niobium in FIG. 3 and 3% niobium in FIG. 4. FIGS. 5 and 6 similarly show the same effect when the chromium content is 30%. FIG. 3 also shows with a broken line the effect of reducing to 1% the niobium con-

tent of alloys containing 10% cobalt and FIG. 4 similarly shows the effect of increasing the niobium content in these alloys to 4%.

The effect of varying the cobalt content is further illustrated by the curves in FIG. 7, in which stress-rupture lives at 3 ton f./in.<sup>2</sup> and 1.8 ton f./in.<sup>2</sup> at 1000° C. are plotted on a logarithmic scale against the cobalt content. The lives at 1.8 ton f./in.<sup>2</sup> at 1000° C. were obtained by extrapolation from results at higher stresses. The broken line relates to alloys nominally containing, apart from cobalt, 25% chromium, 2% niobium, 0.75% carbon and (Mo+½W) 5%, balance nickel, and the full lines to alloys nominally containing 30% chromium, 2% niobium, 0.75% carbon and 6% tungsten, balance nickel.

It will be seen that the best stress-rupture lives were provided by the alloys containing 25% chromium, 12.5% cobalt and 2% niobium at a content of percent Mo+½ (percent W) of from 4% to 7%, and by those containing 30% chromium, 25% cobalt and 2% niobium with percent Mo+½ (percent W) from 2% to 4%.

Table I hereinafter shows the stress-rupture lives obtained other conditions as well as 3 ton f./in.<sup>2</sup> at 1000° C. in alloys having these satisfactory combinations of elements with varying combined molybdenum and tungsten contents. The Charpy V-notch impact strengths of the alloys at 20° C. are also given, some specimens being tested in the as-cast condition and others after being held for 1000 hours at 800° C. to simulate prolonged heating in service and then cooled in air.

TABLE II

| 5  | Alloy No. | (Nominal percent) Nb | Stress-rupture life 1,000° C. at— |                                 | Charpy V-notch impact strength at 20° C. (ft.-lb.) |                              |
|----|-----------|----------------------|-----------------------------------|---------------------------------|----------------------------------------------------|------------------------------|
|    |           |                      | 3.5 ton f./in. <sup>2</sup> (hr.) | 3 ton f./in. <sup>2</sup> (hr.) | As-cast                                            | 1,000 hr./800° C. air-cooled |
|    | A         | 0                    | 64                                | 71                              |                                                    |                              |
|    | 7         | 1                    | 186                               | 300                             | 2.9                                                | 1.5                          |
|    | 1         | 2                    | 186                               | 615                             | 2.9                                                | 1.5                          |
|    | 8         | 3                    | 162                               | 376                             | 2.9                                                | 1.5                          |
| 10 | B         | 6                    | 62                                | 206                             | 2.2                                                | 1.5                          |
|    | C         | 8                    | 28                                | 56                              | 3.6                                                | 2.2                          |

It will be seen that Alloy A, which contained no niobium, gave a very poor result, while Alloys B and C with more than 5% niobium were again poor.

15 The effect of varying the carbon content in alloys otherwise of the composition of Alloy No. 2 is shown by Table III.

TABLE III

| 20 | Alloy No. | Analyzed carbon content (percent) | Stress-rupture life at 1,000° C.  |                                 | Charpy V-notch impact strength at 20° C. (ft.-lb.) |                              |
|----|-----------|-----------------------------------|-----------------------------------|---------------------------------|----------------------------------------------------|------------------------------|
|    |           |                                   | 3.5 ton f./in. <sup>2</sup> (hr.) | 3 ton f./in. <sup>2</sup> (hr.) | As-cast                                            | 1,000 hr./800° C. air-cooled |
|    | D         | 0.36                              | 69                                | 194                             | 5.8                                                | 2.9                          |
|    | 9         | 0.49                              | 94                                | 528                             | 4.3                                                | 2.2                          |
|    | 10        | 0.62                              | 260                               | 660                             | 2.9                                                | 2.2                          |
|    | 11        | 0.70                              | 342                               | 1,019                           | 2.9                                                | 1.5                          |
|    | 2         | 0.77                              | 252                               | 833                             | 2.9                                                | 2.9                          |
|    | 12        | 0.91                              | 291                               | 816                             | 2.2                                                | 1.5                          |
|    | 13        | 1.14                              | 145                               | 440                             | 2.2                                                | 1.5                          |

TABLE I

| Alloy number | Percent |    |    |   |     |    | Combined Mo+½ W (percent) | Stress-rupture life (hr.) |     |       | Impact strength <sup>1</sup> |     |
|--------------|---------|----|----|---|-----|----|---------------------------|---------------------------|-----|-------|------------------------------|-----|
|              | C       | Cr | Co | W | Mo  | Nb |                           | (a)                       | (b) | (c)   | (d)                          | (e) |
| 1            | 0.75    | 25 | 10 | 6 | 1   | 2  | Balance                   | 4                         | 186 | 615   | 661                          | 2.9 |
| 2            | 0.75    | 25 | 10 | 6 | 2   | 2  | do                        | 5                         | 252 | 833   | 956                          | 2.9 |
| 3            | 0.75    | 25 | 10 | 9 | 0.5 | 2  | do                        | 5                         | 397 | 1,080 | 1,184                        | 2.9 |
| 4            | 0.75    | 25 | 10 | 6 | 3   | 2  | do                        | 6                         | 212 | 625   | —                            | 1.5 |
| 5            | 0.75    | 25 | 10 | 6 | 6   | 2  | do                        | 9                         | 111 | 396   | 454                          | 1.5 |
| 6            | 0.75    | 30 | 25 | 6 | —   | 2  | do                        | 3                         | 284 | 1,463 | —                            | —   |

<sup>1</sup> Impact strength or energy in foot-pounds (ft.-lb.).

(a) 3.5 ton f./in.<sup>2</sup> at 1,000° C.

(b) 3.0 ton f./in.<sup>2</sup> at 1,000° C.

(c) 2.0 ton f./in.<sup>2</sup> at 1,050° C.

(d) As-cast.

(e) After heating at 800° C. for 1,000 hr. and air-cooling.

Replacement of the 2% niobium in Alloy No. 3 by 50 4% tantalum reduced the stress-rupture life at 3.5 ton f./in.<sup>2</sup> at 1000° C. to 61 hours and the life at 3.0 ton f./in.<sup>2</sup> at 1000° C. to only 137 hours.

In comparing the results in the tables with the curves in the accompanying drawings, it should be appreciated that the curves are based on the results of a large number of tests and that inevitably there is some scatter of actual test results above and below the curves. This arises both from experimental variation and from the fact that the alloys tested did not all have the same proportions of molybdenum and tungsten. Variation of the proportions of molybdenum and tungsten chiefly affects the optimum stress-rupture life, and this effect is shown by the set of curves in FIG. 8, which relate to alloys nominally containing also 25% chromium, 10% cobalt, 2% niobium, 0.75% carbon and balance nickel. It will be seen that the tungsten-free alloys have relatively poor properties and the stress-rupture lives increase as the proportion of tungsten increases. There is already a substantial improvement when the alloys contain at least 2% tungsten, while the alloys containing at least 5% tungsten are even stronger.

The effect of varying the niobium content in alloys otherwise of the composition of Alloy No. 1 is shown by the stress-rupture and impact test results in Table II. 70

The remarkable improvement in stress-rupture strength in Alloys Nos. 2 and 9 to 13 as compared with Alloy D containing less than 0.4% carbon shows the importance of controlling the carbon content according to the invention.

55 For the purpose of comparison, Table IV shows the composition of, and results obtained with, three commercial alloys that are used or proposed to be used for reformer tubes. The considerable improvement in stress-rupture life obtained by means of the invention is clear from a comparison of Table I with Table IV.

TABLE IV

| 65 | Alloy | Typical stress-rupture properties of commercial alloys <sup>1</sup> |    |    |    |         |                                                                      |
|----|-------|---------------------------------------------------------------------|----|----|----|---------|----------------------------------------------------------------------|
|    |       | Nominal composition (wt. percent)                                   |    |    |    |         | Stress-rupture life at 3 ton f./in. <sup>2</sup> and 1,000° C. (hr.) |
|    | G     | 0.4                                                                 | 25 | 20 | —  | Balance | 17                                                                   |
|    | H     | 0.5                                                                 | 26 | 35 | 15 | 5       | do                                                                   |
|    | J     | 0.5                                                                 | 25 | 50 | —  | 5       | do                                                                   |

<sup>1</sup> Estimated from published data.

The results in Table V show the effects of additions of titanium, zirconium and/or boron and of residual amounts of magnesium added as a deoxidant on the room-temperature tensile properties of alloys with two levels of

carbon and iron contents. Apart from the elements shown in the Table V, the alloys nominally contained 25% chromium, 10% cobalt, 6% tungsten, 2% molybdenum and 2% niobium, balance nickel. In this Table V "N/P" is the ratio of notched to plain tensile strength, "El" is the elongation on a gauge length of 5.65 times the square root of the area, and "R of A" is the reduction in area.

composition, apart from carbon, titanium, zirconium and aluminum in the amounts given in Table VII-A: 25% chromium, 12% cobalt, 9% tungsten, 0.5% molybdenum 2% niobium, 3% iron, balance nickel. The stress-rupture and tensile properties of the alloys, of which Alloys 30 to 34 were in accordance with the invention but Alloy K was not, are set forth in Table VII-A and VII-B.

TABLE V

| Alloy number | Composition (wt. percent analyzed) |    |      |      |       |       |       | R of A<br>(percent) |
|--------------|------------------------------------|----|------|------|-------|-------|-------|---------------------|
|              | C                                  | Fe | Ti   | Zr   | B     | Mg    | N/P   |                     |
| 14           | 0.47                               |    |      |      |       |       | 1.24  | 4.5                 |
| 15           | 0.48                               |    | 0.31 |      |       |       | 1.20  | 13.5                |
| 16           | 0.46                               |    |      | 0.06 |       |       | 1.32  | 9.0                 |
| 17           | 0.47                               |    |      |      | 0.009 |       | 1.30  | 6.8                 |
| 18           | 0.48                               |    |      | 0.06 | 0.009 |       | 1.35  | 5.6                 |
| 19           | 0.50                               |    |      |      |       | 0.02  | 1.25  | 5.6                 |
| 20           | 0.63                               |    |      |      |       |       | 1.16  | 4                   |
| 21           | 0.62                               |    |      |      |       |       | 0.024 | 1.23                |
| 22           | 0.64                               | 3  | 0.11 |      |       | 0.041 | 1.33  | 2.6                 |
| 23           | 0.62                               | 3  | 0.17 |      |       | 0.028 | 1.22  | 6.0                 |
| 24           | 0.64                               | 3  | 0.38 |      |       | 0.028 | 1.17  | 6.0                 |
| 25           | 0.65                               | 3  | 0.8  |      |       | 0.033 | 1.27  | 7.0                 |
| 26           | 0.71                               |    |      |      |       |       | 1.13  | 2.3                 |

Comparison of Alloy 14 with the five following alloys shows respectively the increase in ductility due to titanium (Alloy 15); the improvement in both ductility and notched/plain tensile strength due to zirconium (Alloy 16); the improvement in notched/plain tensile strength due to boron (Alloy 17); the combined effect of zirconium and boron (Alloy 18); and the effect of magnesium (Alloy 19). The undesirable effect of increasing carbon on notched/plain tensile strength ratio and ductility is shown by comparison of Alloys 14, 20 and 26, and the effect of magnesium is also shown by comparison of Alloy 20 and 21. The beneficial effect of zirconium on both

TABLE VII-A

| Alloy number | Percent |      |    |    | Stress-rupture life (hr.) |       |       |       |
|--------------|---------|------|----|----|---------------------------|-------|-------|-------|
|              | C       | Ti   | Zr | Al | (a)                       | (b)   | (c)   | (d)   |
| K            | 0.34    |      |    |    | 79                        | 346   | 440   | 300   |
| 30           | 0.45    |      |    |    | 212                       | 956   | 1,324 | 646   |
| 31           | 0.64    |      |    |    | 301                       | 1,186 | 1,617 | 831   |
| 32           | 0.47    | 0.01 |    |    | 242                       | 1,264 | 2,235 | 825   |
| 33           | 0.45    | 0.1  |    |    | 282                       | 1,681 | 2,091 | 1,078 |
| 34           | 0.42    |      |    |    | 0.44                      |       |       |       |

(a)=3.5 ton f./in.<sup>2</sup> at 1,000° C.(b)=2.7 ton f./in.<sup>2</sup> at 1,000° C.(c)=2.5 ton f./in.<sup>2</sup> at 1,000° C.(d)=2.0 ton f./in.<sup>2</sup> at 1,050° C.

TABLE VII-B

| Alloy number | Tensile properties—as cast       |                              |               |                  | Tensile properties—1,000 hr./1,000° C. |                              |               |                  | Impact strength, ft.-lbs. |
|--------------|----------------------------------|------------------------------|---------------|------------------|----------------------------------------|------------------------------|---------------|------------------|---------------------------|
|              | 0.1% PS, ton f./in. <sup>2</sup> | UTS, ton f./in. <sup>2</sup> | El. (percent) | R of A (percent) | 0.1% PS, ton f./in. <sup>2</sup>       | UTS, ton f./in. <sup>2</sup> | El. (percent) | R of A (percent) |                           |
| K            | 19                               | 38.0                         | 13            | 13               | 17.8                                   | 41.9                         | 11            | 10               | 5.4                       |
| 30           | 18                               | 37.9                         | 12            | 10               | 18.5                                   | 39.9                         | 3.8           | 2.0              | 6.1                       |
| 31           | 19                               | 38.0                         | 6.9           | 6                | 20.9                                   | 41.7                         | 2.2           | 2.0              | 4.7                       |
| 32           | 20                               | 37.5                         | 7.9           | 10               | 20.7                                   | 40.5                         | 2.7           | 2.0              | 7.6                       |
| 33           | 18                               | 39.0                         | 15            | 12               | 19.5                                   | 41.9                         | 5.2           | 5.0              | 8.0                       |
| 34           | 19.3                             | 39.9                         | 11            | 9                |                                        |                              |               |                  | 3.6                       |

PS=Proof stress.

UTS=Ultimate tensile strength.

1,000 hr./1,000° C.=Held for 1,000 hours at 1,000° C. prior to testing at room temperature.

notched/plain tensile strength ratio and ductility are again shown by the results for alloys 22 to 25.

The effect of varying the iron content of the alloys is shown by the results in Table VI, which relate to alloys nominally containing, along with the amounts of iron shown, 0.75% carbon, 25% chromium, 10% cobalt, 6% tungsten, 2% molybdenum and 2% niobium, the balance being nickel.

The weldability of the alloys is surprisingly good, particularly when they contain zirconium or titanium or both and when their carbon content does not exceed 0.65%. The following example of the welding of alloys of the invention illustrates the advantage of the use of a filler material of high zirconium content on the stress-rupture life and elongation of the weld metal.

The centrifugally-cast tubes of Alloys 30 and 32 were cut transversely, the cut ends prepared to a standard J-section and then welded together by argon-shielded arc welding using filler metal of matching composition, which accordingly was zirconium-free in the filler for Alloy 30 and contained 0.01% zirconium in the filler for Alloy 32. In each instance, sound welds were obtained with no evidence of heat-affected zone cracking.

Stress-rupture tests on weld metal deposited from alloys of the same composition as Alloys 30 and 32 and from a third otherwise similar alloy containing 0.48% zirconium produced the following results:

TABLE VI

| Alloy number | Fe (percent) | Stress-rupture life (hr.) |      | Impact strength (ft.-lb.) |     |
|--------------|--------------|---------------------------|------|---------------------------|-----|
|              |              | (A)                       | (B)  | (C)                       | (D) |
| 2            | 0            | 833                       | 956  | 2.9                       | 2.9 |
| 27           | 1.5          | 554                       | 579  | 2.9                       | 2.2 |
| 28           | 3            | 576                       | 612  | 3.6                       | 2.9 |
| 29           | 5            | 341                       | >836 | 2.9                       | 1.5 |

(A)=Stress rupture life at 3.0 ton f./in.<sup>2</sup> at 1,000 degrees C.(B)=Stress rupture life at 2.0 ton f./in.<sup>2</sup> at 1,050 degrees C.

(C)=Impact strength ft.-lb. as cast.

(D)=Impact strength ft.-lb. after 1,000 hrs. at 800 degrees C.

To demonstrate the properties of the alloys when cast in the form of centrifugally cast tubes, six tubes with dimensions of 5-inches outside diameter and 1-inch wall thickness were cast in a commercial centrifugal casting machine. Each of the melts for the tubes was deoxidized by an addition of 0.03 percent magnesium, as nickel-15 percent magnesium alloy, and had the following nominal

| Zr (percent) | Stress-rupture properties at 2.7 ton f./in. <sup>2</sup> , 1,000° C. |                      |
|--------------|----------------------------------------------------------------------|----------------------|
|              | Life (hrs.)                                                          | Elongation (percent) |
| 0            | 152                                                                  | 2.2                  |
| 0.01         | 138                                                                  | 1.2                  |
| 0.48         | 1,166                                                                | 15                   |

While the alloy of the invention is particularly useful for cast reformer tubes and other parts of hydrocarbon reforming plant apparatus, the alloy can also be utilized with advantage for other cast articles and parts of apparatus exposed to stress and corrosive attack at very high temperatures, for example, spinners for the production of glass fibers. Alloys in accordance with the invention can also be worked by conventional hot-working techniques such as rolling, forging and extrusion.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. An alloy consisting essentially of 0.4% to 0.8% carbon, 24% to 27% chromium, cobalt in an amount from 8% to 20% and so correlated with the chromium content that the percentages of cobalt and chromium in the alloy are represented by a point within the area MNOPQM in FIG. 2 of the accompanying drawing, metal from the group consisting of molybdenum, tungsten and mixtures thereof in amounts such that the tungsten content is at least 5% and the sum percent Mo+1/2 (percent W) is 4% to 7%, 1.5% to 2.5% niobium, up to 5% iron, up to 1% of metal from the group consisting of titanium, aluminum and mixtures thereof, up to 1% zirconium, up to 0.1% boron and balance essentially nickel.

2. An alloy according to claim 1 which contains one or both of titanium and zirconium in amounts from 0.03% to 0.2% titanium and 0.005% to 0.3% zirconium.

3. A centrifugally-cast tube made from an alloy according to claim 1 in which the carbon content is 0.43% to 0.65%.

4. A welded structure made from an alloy according

to claim 1 in which the carbon content does not exceed 0.65% and which contains titanium or zirconium or a mixture thereof.

5. An alloy according to claim 1 containing about 25% chromium, about 12% cobalt, about 9% tungsten, about 0.5% molybdenum, about 2% niobium, either about 0.1% titanium or about 0.01% zirconium, and about 3% iron.

#### References Cited

##### UNITED STATES PATENTS

|           |         |                  |           |
|-----------|---------|------------------|-----------|
| 3,212,886 | 10/1965 | Freedman         | 75—171    |
| 2,513,469 | 7/1950  | Franks et al.    | 75—171 X  |
| 2,537,477 | 1/1951  | Mohling et al.   | 75—171 X  |
| 2,543,841 | 3/1951  | Foley            | 75—171 X  |
| 3,069,258 | 12/1962 | Haynes           | 75—171 UX |
| 3,127,265 | 3/1964  | Avery            | 75—171    |
| 3,316,074 | 4/1967  | Laurent et al.   | 75—171 X  |
| 3,368,889 | 2/1968  | Baumel           | 75—171    |
| 3,508,917 | 4/1970  | Fleetwood et al. | 75—171    |
| 3,411,899 | 11/1968 | Richards et al.  | 75—171    |
| 3,466,171 | 9/1969  | Fletcher et al.  | 75—171    |
| 3,493,366 | 2/1970  | Hopkins          | 75—171 X  |
| 3,552,952 | 1/1971  | Shaw             | 75—171    |

##### FOREIGN PATENTS

|         |         |                |
|---------|---------|----------------|
| 654,354 | 6/1951  | Great Britain. |
| 637,436 | 5/1950  | Great Britain. |
| 612,001 | 11/1948 | Great Britain. |
| 773,871 | 5/1957  | Great Britain. |
| 617,194 | 2/1949  | Great Britain. |
| 674,023 | 6/1952  | Great Britain. |
| 681,247 | 10/1952 | Great Britain. |

HENRY W. TARRING II, Primary Examiner

U.S. Cl. X.R.

75—171; 148—32

UNITED STATES PATENT OFFICE  
CERTIFICATE OF CORRECTION

Patent No. 3,681,059

Dated August 1, 1972

Inventor(s) Stuart Walter Ker Shaw and Peter John Penrice

It is certified that error appears in the above-identified patent  
and that said Letters Patent are hereby corrected as shown below:

Column 3, line 47, for "MUVPQM" read --MUVPQM--.

Column 4, line 6, for "deoxidized" read --deoxidized--.

Column 7, line 32, delete "boron (Alloy 18);

and the effect of magnesium (Alloy".

Signed and sealed this 7th day of May 1974.

(SEAL)

Attest:

EDWARD M. FLETCHER, JR.  
Attesting Officer

C. MARSHALL DANN  
Commissioner of Patents